

Sept. 4, 1951

J. R. FISHER, JR

2,567,106

METHOD OF TREATING OILS

Filed Sept. 6, 1946

3 Sheets-Sheet 1



Sept. 4, 1951

J. R. FISHER, JR

2,567,106

METHOD OF TREATING OILS

Filed Sept. 6, 1946

3 Sheets-Sheet 2



Sept. 4, 1951

J. R. FISHER, JR

2,567,106

## METHOD OF TREATING OILS

Filed Sept. 6, 1946

3 Sheets-Sheet 3



FIG. 3

INVENTOR  
JOHN R. FISHER JR.

BY  
*Toulmin & Toulmin*  
ATTORNEYS

## UNITED STATES PATENT OFFICE

2,567,106

## METHOD OF TREATING OILS

John R. Fisher, Jr., Dayton, Ohio, assignor to The Commonwealth Engineering Company of Ohio, Dayton, Ohio, a corporation of Ohio

Application September 6, 1946, Serial No. 695,211

4 Claims. (Cl. 260—407)

1

This invention deals with a method of treating oils, and in particular with a method of bodying drying oils.

It is an object of this invention to provide a method of treating drying oils in which an increase of viscosity may be obtained in a very short period of time.

It is another object of this invention to provide a method of treating drying oils by which oils are obtained that have the advantageous properties of conventionally heat-bodied and of air-blown oil combined.

It is another object of this invention to provide drying oils which, when mixed with the customary ingredients for composing a varnish, yield varnishes which dry to an extremely tough and highly flexible coating.

It is still another object of this invention to provide a drying oil which, when admixed with the usual ingredients, yields varnishes which are extremely fast drying.

These and other objects are accomplished by exposing the oils to a high frequency field.

In carrying out the method of my invention, the oil is placed into a non-conductive container, and two electrodes, for example copper electrodes, are inserted therein. The electrodes are connected with a high frequency oscillator, and the oil is thus subjected to a high frequency field. The frequency and the intensity of the current are not critical; however, a current of substantially 9 megacycles and 0.7 ampere was found most satisfactory. The oils were treated for two hours in each case, and samples for determining the viscosity were taken every ten minutes. In each case, for the sake of comparison, an experiment was also carried out in which the oil was subjected to the conventional heat-bodying processes.

In the following tables, the results of some of the treatments by the process of my invention are compiled. Table 1A gives the results of viscosity measurements, in poises, made every ten minutes with high-frequency treated China wood oil and Table 1B the corresponding results with conventionally heat-treated China wood oil. Tables 2A and 2B give the analogous results for castor oil and Tables 3A and 3B those for oiticica oil.

2  
TABLE 1A  
CHINA-WOOD OIL—HIGH FREQUENCY TREATMENT

| Heating Time | Temperature of Oil | Viscosity in Poises |
|--------------|--------------------|---------------------|
| Min.         | °F.                |                     |
| 10           | 199                | 4.35                |
| 20           | 243                | 4.35                |
| 30           | 262                | 4.35                |
| 40           | 253                | 4.44                |
| 50           | 280                | 4.44                |
| 60           | 275                | 4.53                |
| 70           | 262                | 4.53                |
| 80           | 230                | 4.62                |
| 90           | 293                | 4.70                |
| 100          | 302                | 4.85                |
| 110          | 302                | 5.00                |
| 120          | 290                | 5.00                |

TABLE 1B  
CHINA-WOOD OIL—CONVENTIONAL HEAT TREATMENT

| Heating Time | Temperature of Oil | Viscosity in Poises |
|--------------|--------------------|---------------------|
| Min.         | °F.                |                     |
| 10           | 275                | 2.81                |
| 20           | 253                | 3.85                |
| 30           | 247                | 4.08                |
| 40           | 260                | 4.08                |
| 50           | 267                | 4.35                |
| 60           | 262                | 4.43                |
| 70           | 273                | 4.43                |
| 80           | 263                | 4.51                |
| 90           | 267                | 4.51                |
| 100          | 273                | 4.51                |
| 110          | 275                | 4.70                |
| 120          | 290                | 4.70                |

TABLE 2A  
CASTOR OIL—HIGH FREQUENCY TREATMENT

| Heating Time | Temperature of Oil | Viscosity in Poises |
|--------------|--------------------|---------------------|
| Min.         | °F.                |                     |
| 10           | 241                | 6.08                |
| 20           | 243                | 6.27                |
| 30           | 255                | 8.84                |
| 40           | 255                | 8.84                |
| 50           | 262                | 8.84                |
| 60           | 265                | 9.30                |
| 70           | 240                | 9.30                |
| 80           | 260                | 9.30                |
| 90           | 255                | 9.76                |
| 100          | 265                | 9.76                |
| 110          | 247                | 9.76                |
| 120          | 260                | 10.70               |

TABLE 2B  
CASTOR OIL—CONVENTIONAL HEAT TREATMENT

| Heating Time | Temperature of Oil | Viscosity in Poises |
|--------------|--------------------|---------------------|
| Min.         | °F.                |                     |
| 10           | 285                | 6.27                |
| 20           | 285                | 6.66                |
| 30           | 257                | 8.84                |
| 40           | 265                | 8.84                |
| 50           | 264                | 8.84                |
| 60           | 262                | 8.84                |
| 70           | 284                | 8.84                |
| 80           | 250                | 8.84                |
| 90           | 265                | 8.84                |
| 100          | 265                | 8.84                |
| 110          | 265                | 8.84                |
| 120          | 257                | 8.84                |

TABLE 3A  
OTICICA OIL—HIGH FREQUENCY TREATMENT

| Heating Time | Temperature of Oil | Viscosity in Poises |
|--------------|--------------------|---------------------|
| Min.         | °F.                |                     |
| 10           | 240                | 4.40                |
| 20           | 263                | 5.50                |
| 30           | 247                | 6.27                |
| 40           | 282                | 7.06                |
| 50           | 275                | 7.06                |
| 60           | 279                | 7.06                |
| 70           | 262                | 7.06                |
| 80           | 275                | 8.84                |
| 90           | 247                | 8.84                |
| 100          | 265                | 8.84                |
| 110          | 265                | 10.70               |
| 120          | 262                | 10.70               |

TABLE 3B  
OTICICA OIL—CONVENTIONAL HEAT TREATMENT

| Heating Time | Temperature of Oil | Viscosity in Poises |
|--------------|--------------------|---------------------|
| Min.         | °F.                |                     |
| 10           | 230                | 5.88                |
| 20           | 257                | 5.88                |
| 30           | 273                | 6.27                |
| 40           | 280                | 6.27                |
| 50           | 264                | 6.27                |
| 60           | 253                | 6.27                |
| 70           | 262                | 6.27                |
| 80           | 265                | 6.27                |
| 90           | 270                | 6.27                |
| 100          | 273                | 7.05                |
| 110          | 270                | 7.05                |
| 120          | 270                | 7.05                |

In the accompanying drawings, these tests and their results are graphically illustrated. In Figure 1, the treatment of China wood oil is shown, an illustration A thereof gives the function of treating time and viscosity in poises for both the high frequency and the conventional heat treatment. It will be seen from this diagram that the high frequency treatment in each instance yields an oil of a higher viscosity. In the diagrams B and C, the temperature factor is also considered. There, the function between temperature and treating time is shown in full lines, and the corresponding viscosity in each case is indicated in broken lines. It is obvious that the curve in diagram C progresses towards a high viscosity in a shorter period of time than does the curve of diagram B.

Figure 2 demonstrates the results of the same treatment, but with raw castor oil. There, the difference between the two processes is even more pronounced. Diagram 2B shows that after approximately 90 minutes the viscosity comes

to a standstill as shown by a plurality of broken lines terminating at the one point of the viscosity 8.84. In contradistinction thereto, the high frequency treatment continuously increases the viscosity, and after two hours it arrives at 10.7 poises.

The best results were obtained with oticica oil, which is the oil used in the instance of Figure 3. The diagram 3A, after a two hours' treatment, shows a difference of viscosities from 7 to almost 11 for the conventionally treated oil and the oil treated according to the invention, respectively.

The process of my invention was found to be operative for all drying oils. The time required for obtaining a predetermined viscosity is considerably reduced and consequently also the cost of such oils. Moreover, the oils treated by the high-frequency method have qualities superior to those heat-bodied in the conventional manner. This is especially obvious in varnishes which have been made from the oils obtained by the process of my invention. Such varnishes derived from oils of my invention are extremely tough and flexible. This feature of high flexibility is particularly important if the varnish is to be applied to flexible base materials, for instance for manufacturing oilcloth. A further advantage of the new method is that the oils can be stored for a practically unlimited period of time without the risk of solidification. This is valuable particularly in the case of oticica oil which, when treated otherwise by any of the conventional methods, solidifies in a very short time and thus becomes worthless during storage.

One of the varnishes made from the oils prepared by the method of the invention and found highly satisfactory is the following:

40

*Example*

100 pounds rosin-modified phenol formaldehyde resin  
10 pounds lead acetate  
25 gallons high frequency treated oticica oil  
45 30 gallons mineral spirits.

The varnish obtained from the above mixture was applied to the base material and then baked at 200° F. for 1 hour and thereafter baked under 50 infrared light for 15 minutes. The coating obtained was very tough and durable and showed a high degree of flexibility.

It will be understood that while there have been described herein certain specific embodiments of the invention, it is not intended thereby to have it limited to or circumscribed by the details given, since the invention is susceptible to various modifications and changes which come within the spirit of the disclosure and the scope 60 of the appended claims.

I claim:

1. In a method of treating fatty vegetable drying oils, the step of exposing the oil to a high-frequency electric field of substantially 9 megacycles and 0.7 ampere for two hours.
2. In a method of treating oticica oil, the step of exposing the oil to a high-frequency electric field of substantially 9 megacycles and 0.7 ampere for two hours.
3. In a method of treating China wood oil, the step of exposing the oil to a high-frequency electric field of substantially 9 megacycles and 0.7 ampere for two hours.
4. In a method of treating castor oil, the step 75 of exposing the oil to a high-frequency electric

## 5

field of substantially 9 megacycles and 0.7 ampere for two hours.

JOHN R. FISHER, JR.

## REFERENCES CITED

The following references are of record in the file of this patent:

## UNITED STATES PATENTS

| Number    | Name          | Date           |    |
|-----------|---------------|----------------|----|
| 2,167,726 | Richardson    | Aug. 1, 1939   | 10 |
| 2,257,177 | Luster        | Sept. 30, 1941 |    |
| 2,268,002 | Waldie        | Dec. 30, 1941  |    |
| 2,364,790 | Hemming       | Dec. 12, 1944  |    |
| 2,411,767 | Waldie et al. | Nov. 26, 1946  | 15 |
| 2,418,451 | Auer          | Apr. 8, 1947   |    |
| 2,446,557 | Schutz et al. | Aug. 10, 1948  |    |

## 6

## FOREIGN PATENTS

| Number  | Country       | Date         |
|---------|---------------|--------------|
| 508,913 | Great Britain | July 7, 1939 |

## OTHER REFERENCES

Ellis, Hydrogenation of Org. Substance, Van Nostrand, 3d ed. 1930, pp. 616-624.  
 Kirchrath, Il H. Seifensieder-Ztg. 1938, 65, pp. 682-683.  
 Zelenin, Maslobino Zhirovoe Delo, 16 No. 4, 16-23 (1940), C. A. 1941, 919.  
 Olive, T. R., Chem. & Met. Eng. April 1943 pp. 102-104.  
 Industrial & Eng. Chem. 36, 1944, pp. 440-447.